

1

2,786,754

**ALLOY COMPOSITION**

John V. Klochkov, New York, N. Y.

No Drawing. Application February 10, 1953,  
Serial No. 336,197

1 Claim. (Cl. 75—134)

This invention relates to a new and improved alloy composition, more particularly an alloy composition which simulates in appearance a precious metal such as gold.

The alloy according to the invention consists of the following metals by weight:

|          | Percent |
|----------|---------|
| Tungsten | 37.1    |
| Tin      | 24      |
| Copper   | 12.8    |
| Cobalt   | 5.9     |
| Mercury  | 20.2    |

2

My new alloy composition yields gold-like alloys which are valuable metallurgical compounds, and which are fully equivalent for industrial purposes, such as in the production of machinery and instruments, especially those in the medical and dental fields, to the precious metals themselves. Because of their simulations of the metal gold, my new metallurgical composition can be used to replace the precious metals, and have very extensive fields of usefulness where formerly gold was employed.

I claim:

An alloy consisting of the following metals by weight:

|          | Percent |
|----------|---------|
| Tungsten | 37.1    |
| Tin      | 24      |
| Copper   | 12.8    |
| Cobalt   | 5.9     |
| Mercury  | 20.2    |

No references cited.